



US008304150B1

(12) **United States Patent**  
**Eberlein et al.**

(10) **Patent No.:** **US 8,304,150 B1**  
(45) **Date of Patent:** **Nov. 6, 2012**

(54) **ELECTROSTATIC PRINTING OF  
FUNCTIONAL TONER MATERIALS FOR  
THE CONSTRUCTION OF USEFUL  
MICRO-STRUCTURES**

(75) Inventors: **Dietmar C. Eberlein**, Wappingers Falls, NY (US); **Robert H. Detig**, New Providence, NJ (US)

(73) Assignee: **Electrox Corporation**, Denville, NJ (US)

(\*) Notice: Subject to any disclaimer, the term of this patent is extended or adjusted under 35 U.S.C. 154(b) by 1352 days.

(21) Appl. No.: **11/752,109**

(22) Filed: **May 22, 2007**

**Related U.S. Application Data**

(60) Provisional application No. 60/802,344, filed on May 22, 2006.

(51) **Int. Cl.**  
**G03G 13/32** (2006.01)

(52) **U.S. Cl.** ..... **430/49.1**; 430/114; 430/124.1

(58) **Field of Classification Search** ..... 430/49.1,  
430/114, 124.1, 137.22

See application file for complete search history.

(56)

**References Cited**

**U.S. PATENT DOCUMENTS**

|                 |         |                      |           |
|-----------------|---------|----------------------|-----------|
| 4,318,002 A *   | 3/1982  | Pressman et al. .... | 250/492.2 |
| 4,990,416 A *   | 2/1991  | Mooney .....         | 430/26    |
| 6,250,984 B1    | 6/2001  | Jin et al.           |           |
| 6,781,612 B1 *  | 8/2004  | Detig .....          | 347/112   |
| 6,815,130 B2 *  | 11/2004 | Eberlein et al. .... | 430/49.1  |
| 2002/0130353 A1 | 9/2002  | Lieber et al.        |           |
| 2004/0173506 A1 | 9/2004  | Doktycz et al.       |           |

\* cited by examiner

*Primary Examiner* — Thorl Chea

(74) *Attorney, Agent, or Firm* — Steven M. Hoffberg; Ostrolenk Faber LLP

(57) **ABSTRACT**

A method for building microstructures, comprising the steps of forming a photopolymer mask on a substrate, having a mask thickness equal to or larger than a desired height of a microstructure to be formed; forming a latent image on the photopolymer mask by exposure to light; applying an electrical charge to the photopolymer mask; developing the cavities in the mask with a functional liquid toner material whose electrical charge polarity is the same as the charge on the mask; and solidifying the functional liquid toner material into a useful microstructure.

**24 Claims, 21 Drawing Sheets**

FIG. 1

Prior Art



FIG. 2 Prior Art



**FIG. 3A** Prior Art  
EXPOSE



**FIG. 3B** Prior Art  
CHARGING



**FIG. 3C** Prior Art  
DELAY



**FIG. 3D** Prior Art  
LIQUID TONER  
DEVELOPMENT



**FIG. 4A** Prior Art**FIG. 4B** Prior Art**FIG. 4C** Prior Art**FIG. 4D** Prior Art



**Fig. 5A**  
Prior Art



**Fig. 5B**  
Prior Art

**FIG. 6A**  
Prior Art



**FIG. 6B**  
Prior Art



**FIG. 6C**  
Prior Art



**FIG. 6D**  
Prior Art





**Fig. 7A**

Prior Art



**Fig. 7B**

Prior Art



**FIG. 9**  
Prior Art



**FIG. 10A**  
Prior Art



**FIG. 10B**  
Prior Art





**FIG. 12**

Prior Art



**FIG. 13A**  
Prior Art



**FIG. 13B**  
Prior Art



**FIG. 13C**  
Prior Art



**FIG. 14A**  
Prior Art



**FIG. 14B**  
Prior Art



**FIG. 14C**  
Prior Art



**FIG. 14D**

Prior Art



## ELECTROSTATIC WAFER BUMPING PROCESS

FIG. 15A Fully Functional Silicon Wafer



FIG. 15B Coat with Photopolymer Mask



FIG. 15C

Pattern Mask



Charge Patterned Mask

FIG. 15D



FIG. 15E Develop with Solder Toner



FIG. 15F Re-flow Toner into Bumps





## BUILDING PLASMA PANEL RIBS



FIG. 17



FIG. 18



Fig. 1a

**ELECTROSTATIC PRINTING OF  
FUNCTIONAL TONER MATERIALS FOR  
THE CONSTRUCTION OF USEFUL  
MICRO-STRUCTURES**

**BACKGROUND OF THE INVENTION**

**1. Field of the Invention**

The invention concerns a process for the electrostatic printing of functional materials, for example conductors or semiconductors, configured as liquid toners for various manufacturing applications.

**2. Description of the Related Art**

**A. Solder Bumping**

Present industry road maps for silicon chips specify 4,000 I/O connections on a chip as small as 15 mm by 15 mm. Since the traditional wire bonding techniques cannot handle this density, wafer bumping or “flip chip” technology is necessarily applied. Each I/O pad requires a relatively tall solder bump, which will make contact eventually with a printed wiring structure. There are three techniques currently used to build these bumps:

1. Stencil printing of solder filled paste. For relatively large features (above 150 micron pad diameter) this method is preferred, since it is simple and requires no additional processing.

2. Flip Chip Technologies Inc. of Phoenix, Ariz. practices a variation of stencil printing, in which a stencil mask is spin coated on the wafer, then photo-lithographically patterned. The electrode cavities are filled with solder ink using a doctor blade. The solder ink is re-flowed into near perfect spheres, and then the mask is stripped chemically.

3. A similar mask is employed as in a doctor blade approach. Problems of this method include a 40 minute plating process to form the bumps, and the difficulty and/or inability to effect a plating of lead free alloys, e.g., Sn/Ag/Cu.

**B. Building Glass Ribs and Other Microstructures**

Plasma display panels are a growing flat panel display technology whose market acceptance has been limited by high manufacturing costs. Two important, high cost elements of this technology include:

- A. Glass barrier ribs, which isolate discharge chambers from one another; and
- B. Electrical lines, usually made of a silver/glass mixture, that is sintered in the 500+° C. range.

The glass barrier ribs were screen printed, but with as many as seven print steps to achieve the 100 microns of needed rib height. Recently, sand blasting techniques have been used, but the costs are still high. The conductive lines are typically photo-defined, with the unexposed materials etched away, causing a large waste of expensive silver which should then be re-cycled.

Field emission displays are a relatively new technology. They consist of an array of field emission points in a vacuum, spraying electrons onto a phosphor screen. With three color dots on the screen and addressability of the emitting points, one has a full color display.

Active matrix liquid crystal displays have been intensively developed for production. The manufacturing process includes: a. photolithography or the patterning of photo sensitive resists and the “washing” and etching processes that are attendant to them, b. printing relatively large area features (30μ or more) c. the low pressure sputtering processes for coating glasses with metals like aluminum or indium/tin oxide (ITO), a transparent electrode or dielectrics like SiO<sub>2</sub>. In all cases the process has many steps, many in which the

substrate glass has to be heated and then cooled back to room temperature before the next step.

See, U.S. Pat. Nos. 6,876,370, 6,781,612, 6,743,319, 6,524,758, 6,379,745, 6,274,412, 6,153,348, 6,143,356, and 5,882,722, each of which is expressly incorporated herein by reference.

Electrostatic printing has been used for color proofing in Du Ponts EMP process during the late 1980’s. Du Pont used the electrostatic printing which is described by Reisenfield in U.S. Pat. No. 4,732,831. It used liquid toners that were transferred directly to a smooth, coated sheet of paper.

The transfer of liquid toner, which is important to this invention, was disclosed by Bujese in U.S. Pat. No. 4,879,184 and U.S. Pat. No. 4,786,576. These documents teach the transfer of liquid toners across a finite mechanical gap, typically 50μ to 150μ. This technology has been applied where toner, with etch resist properties, was transferred to copper clad glass epoxy boards.

Other prior work related to the printing plate and “gap transfer” includes M. B. Culhane (Defensive Publication# T869004, Dec. 16, 1969) and Ingersol and Beckmore to the electrostatic printing plate (See, U.S. Pat. Nos. 3,286,025, RE 29,357; and RE 29,537, respectively).

**SUMMARY OF THE INVENTION**

One aspect of the present invention provides an electrostatic printing process for the building of microstructures on suitable substrates. A photopolymer mask may be used, patterned in the shape of the microstructure to be formed. A developing process puts functional toner material in a liquid in the cavities formed in the mask. After an optional processing step to stabilize the microstructure, the mask may be optionally stripped away, for example by chemical means.

Briefly described, one aspect of the invention provides a technique for the electrostatic printing of functional materials on glass to produce various “microstructures” like ribs or electrodes, spacers, filters etc. by machine similar to a copy machine or laser printer at rates from 0.1 to 1.0 msec, and possibly higher. In some cases there is a later step of sintering or electro-less plating, but this is “after the fact”, in that dimensional accuracy was previously determined by the printing step done at generally room temperature. The functional materials include metals, dielectrics, phosphors, catalytic seed materials, etc. configured as liquid toners. For example, fine particulates are suspended in a dielectric fluid. Since a preferred substrate material is glass, it presents special requirements: (1) It may be mechanically of irregular shape (i.e. wedge shaped in orthogonal directions and its thickness has considerable variation); and, (2) It may be a very thick material to be electrostatically imaged compared to the paper or polymeric films printed on by copiers or laser printers.

The present invention therefore preferably uses liquid toners (dispersions of solid particles; metal, glass, etc.) that can be electrostatically transferred across a significant mechanical fluid filled gap.

While the “gap transfer” technique is useful in production machinery handling 1.0 m by 1.4 m plates, there are many situations where the printing capability on a relieved surfaced is a significant advantage, and the magnitude of surface relief can be quite substantial, of the order of 0.1 mm or 100μ or more.

The electrostatic printing function is typically done in one process step. Afterwards, the particulate mass may be fused into a solid structure with a subsequent heating step. In one embodiment of the invention, catalytic seed toners are printed

followed by "electroless" plating steps where metals like copper, or nickel, are deposited on the glass.

There are certain partially manufactured products like color filters or CRT face plates which can be used in a process wherein the final part plays the role of a printing plate to print on itself. This is very simple and therefore inexpensive process which contains a "self-healing" feature. Imperfections in the semi finished parts are automatically overprinted with the liquid toner.

It is therefore an object according to the present invention to provide a method for building microstructures, comprising the steps of: forming a patterned dielectric mask on a substrate, having a mask thickness equal to or larger than a desired height of a microstructure to be formed, and relief features formed into the mask; applying an electrical charge to the patterned dielectric mask, to thereby form a spatial charge pattern; developing the charge pattern with electro-chemically charged functional toner in a liquid; and processing the functional toner material to form a useful microstructure corresponding to the relief features of the patterned dielectric mask.

The functional toner may comprise a first portion of higher melt point glass mixed with a second portion of a lower melt point material, which re-flows and bonds the higher melt point material together, while still retaining the original shape of the structure after processing. Preferably, the first portion is present in a greater quantity than the second portion, the first and second portions comprising a majority of a solids portion of the functional toner.

The functional toner may also comprise metal particles coated with an organic-metallic composition suspended in a liquid. The processing step, in this case, preferably comprises decomposing the organic-metallic composition under heat, to leave a metal product, which will sinter the particles together, wherein the sintered particles correspond to the mask in shape.

Likewise, the functional toner may comprise inorganic (or organic) particles coated with an organic-metallic composition suspended in a liquid, wherein the processing step comprises heating to decompose the organic-metallic composition, the decomposition product of the heated organic-metallic composition sintering the inorganic (or organic) particles together, wherein the metal particles correspond in shape to the mask.

The functional toner may comprises particles, each comprising a particle core composition coated with a particle shell composition, the particle shell composition transforming in the processing step to form a solid matrix with the particle core composition, wherein the solid matrix corresponds in shape to the mask. By way of example, and not limitation, the shell composition may alloy with the core, and as a result, lower its melting point, so that the ambient conditions melt the alloyed portion under sintering conditions. The particle shell composition may also transform into the same or a different composition as the particle core, for example by decomposition of an appropriate organo-metallic composition. Likewise, the shell composition may decompose to form a "sticky" composition which adheres to the core composition and decomposition product. Further, the shell composition may react with a chemical in the environment, to solidify.

The processing step may comprise exposing the developed functional toner material to one or more of actinic radiation, an exogenous chemical, and heat, to initiate or maintain a decomposition or polymerization reaction. The particles, or a portion thereof, may undergo a temporary or permanent phase transformation between solid, liquid and/or gas (i.e., melting, freezing, vaporization, sublimation, condensation,

etc.). For example, the processed functional toner may comprise a material having a reflow temperature, wherein the functional toner is reflowed to form spheres due to surface tension forces. For most solder materials, the surface tension is sufficient to form near-perfect spheres, especially if not particularly confined on the exposed areas and with a relatively small substrate adhesion portion, i.e., a portion of the substrate which is wetted by the solder. Further, in addition to the patterned dielectric mask, a solder mask may be formed on the substrate, to limit the portions of the substrate which can be wetted by the reflowed functional toner material. Preferably, this solder mask is also dielectric.

A preferred toner comprises a solder, for example containing tin and optionally one or more of lead, silver, copper, antimony, bismuth, gallium, cadmium, indium and/or zinc. More preferred are solders which comply with the European Union RoHS directive, which precludes, for example, lead and cadmium from forming significant portions of the composition. It is noted that the processed toner composition of the present invention may be homogeneous or heterogeneous, for example layered, or have residual particle inhomogeneities, and thus, even under reflow conditions which normally produce a homogeneous melt, only a portion of the useful structure may actually reach such a temperature. This, in turn, may produce mechanical barriers within the microstructure to tin whisker elongation. Likewise, the residual particulates may form alloys with tin inclusions over time (which do not form immediately due to the controlled process temperatures) which prevent the tin whisker growth.

According to a further embodiment of the invention, the functional toner comprises particles having a core having a high melting temperature, a mantle having a low melting temperature, and a crust having surfactant properties, wherein the processing step removes at least a portion of the crust and maintains a temperature between a melting temperature of the mantle and the crust, to thereby adhere the functional toner particles into a matrix.

The microstructure may be, for example, a solder bump, a rib or a barrier. For example, the spatial charge pattern may define at least one rib having a length preferably three, and more preferably ten times longer than a width thereof. The spatial charge pattern may define at least one barrier at least partially surrounding a feature of the substrate. The microstructure may also be a micromechanical device, such as a cantilever, gear, electrical brush, electrical sensor, gravitational sensor (accelerometer), chemical sensor, or the like. The microstructure may form an electrical device such as an inductor, antenna, capacitor, resistor, transistor, diode, light emitter, photosensor, thermosensor, chemi-sensor, or the like.

The functional toner material may comprise a glass type frit, wherein the processing step fuses the frit into a glass type structure on the substrate.

The process is capable of producing microstructures having a section height greater than a respective section width. Thus, tall aspect ratios are available. This is advantageous, for example, in making barriers, closely-spaced conductors (e.g., metallic), sensors, and the like. Depending on the toner particulate composition, electrical charge patterns, and processing conditions, process may produce aspect ratios (H/W) of 2:1 or higher. In the case of a solder bump, a 1:1 ratio is anticipated due to the sphericity.

According to another aspect of the invention, the substrate may be non-planar, and the resulting processed microstructures formed on the substrate are also non-planar. Likewise, the processed microstructures may be stacked, e.g., the substrate comprises existing microstructures, and wherein the processed microstructures are formed superposed on the

## 5

existing microstructures, provided the underlying structure has sufficient electrical conductivity that it cannot hold charge.

A particular aspect of the invention permits microstructures having differing compositions to be formed. Thus, the substrate may comprise existing microstructures formed of a first processed functional toner type, and wherein the processed microstructures are formed of a second processed functional type, to thereby product a plurality of processed microstructures having different material compositions. Again the underlying materials must be of sufficient conductivity that they are unable to hold electrical charge.

The substrate may comprise a plurality of electrodes, wherein the electrodes can be selectively excited, to perform a process comprising: first: applying an electrical charge to a first electrode, to thereby form a first spatial charge pattern in proximity thereto; developing the first charge pattern with electrically charged first functional toner in a liquid; and processing the developed first functional toner corresponding to the first charge pattern to form a first useful microstructure corresponding to the relief features of the patterned dielectric mask in proximity to the first electrode; and second: applying an electrical charge to a second electrode, to thereby form a second spatial charge pattern in proximity thereto; developing the second charge pattern with electrically charged second functional toner in a liquid; and processing the developed second functional toner material corresponding to the second charge pattern to form a second useful microstructure corresponding to the relief features of the patterned dielectric mask in proximity to the second electrode, wherein the first useful microstructure and second useful microstructure are formed of different toner compositions.

Alternately, the developing step may comprise partially developing the charge pattern with electrically charged first functional toner in a liquid; and then partially developing the charge pattern electrically charged second functional toner in a liquid, to thereby produce useful microstructures having varying compositions. The developing step may comprise partially developing the charge pattern with electrically charged first functional toner in a liquid to incompletely fill the patterned mask; and then developing the charge pattern electrically with electrically charged second functional toner in a liquid to finish filling the patterned mask, to thereby produce a layered useful microstructure, provided that the first layer of toner is of a conductive material such that it does not hold charge.

This is accomplished by successively increasing the driving voltage (effectively the voltage level on the mask) with each additional imaging step.

Further, the charge on the patterned mask can be selectively applied according to a plurality of distributions, the process comprising the steps of applying a first spatial charge distribution to the patterned mask; developing the first spatial charge pattern with electrically charged first functional toner in a liquid; optionally at least partially processing the first functional toner prior to developing with the second functional toner; applying a second spatial charge distribution to the patterned mask; developing the second spatial charge pattern with electrically charged second functional toner in a liquid, superposed on the developed first functional toner; processing the superposed first and second functional toner to form a useful microstructures, wherein a composition of the microstructures varies in dependence on the first and second spatial charge distributions. The first functional toner and second functional toner may be processed to form a useful microstructure having, at any location, a homogeneous composition or a heterogeneous composition. For example, the

## 6

processing step may vary regionally, for example by zoned heating, masking of actinic radiation, selective ion beam irradiation, etc.

Typically, the functional toner in a liquid comprises particles having a charge of the same polarity as the electrical charge applied to the patterned dielectric mask. The charge may be applied from the front (exposed) surface, or from behind. An important aspect of the invention is that the pattern mask, in conjunction with the charging step, produce and maintain during the process a spatially patterned charge distribution which will selectively cause the charged liquid toner to selectively migrate according to the relief structures during the toner development process. Thus, the electrostatic forces of the charged mask and the charged liquid toner are active to apply a force on the toner material into the crevices.

The patterned dielectric mask may optionally be removed, preferably without disturbing the formed useful microstructure.

20 The substrate may also be a thin dielectric, wherein the process further comprises providing a conductor on an opposite side of the substrate from the dielectric mask, and imposing a charge on the conductor, to thereby form the spatial charge pattern.

25 The developing step may comprise partially developing the charge pattern with electrically charged first functional in a liquid; and then partially developing the charge pattern with electrically charged second functional toner in a liquid, to thereby produce a useful microstructures having varying 30 compositions.

35 The charge on the patterned mask can be a lied according to a plurality of distributions, the process comprising the steps of: applying a first spatial charge distribution to the patterned mask; developing the first spatial charge pattern with electrically charged first functional toner in a liquid; applying a second spatial charge distribution to the patterned mask; developing the second spatial charge pattern with electrically charged second functional toner in a liquid, superposed on the developed first functional toner; and processing the superposed first and second functional toner to form a useful microstructures wherein a composition of the microstructures varies in dependence on the first and second spatial charge distributions.

40 The developed first functional toner may be at least partially processed prior to developing with the second functional toner.

45 The developing step may comprise partially developing the charge pattern with electrically charged first functional toner in a liquid to incompletely fill the patterned mask; and then developing the charge pattern electrically charged second functional toner in a liquid to finish filling the patterned mask, to thereby produce a layered useful microstructure.

50 The process may further comprise the step of removing the patterned dielectric mask without disturbing the formed useful microstructure.

55 The substrate may be a thin dielectric, the process further comprising providing a conductor on an opposite side of the substrate from the dielectric mask, and imposing a charge on the conductor, to thereby form the spatial charge pattern.

60 The spatial charge pattern may define at least one barrier at least partially surrounding a feature of the substrate.

The substrate may comprise existing microstructures, and the processed microstructures may be formed superposed on the existing microstructures.

65 The substrate may comprise existing microstructures formed of a first processed functional toner type, and the processed microstructures may be formed of a second pro-

cessed functional type, to thereby produce a plurality of processed microstructures having different material compositions.

The invention may be more fully understood by referring to the following drawings.

#### BRIEF DESCRIPTION OF THE DRAWINGS

FIG. 1 illustrates an overall mechanical schematic of the invention.

FIG. 2 illustrates a detailed view of the nip between drum and glass.

FIGS. 3A-D illustrate the electrostatic printing plate and the four steps in the imaging process.

FIGS. 4A-C illustrate the progressive exposure of the electrostatic printing plate.

FIG. 4D illustrates a plate exposed one quarter of its thickness.

FIGS. 5A-B illustrates the ideal and typical charge decay curves for the electrostatic printing plate.

FIGS. 6A-D illustrates the four typical corona devices used in copy machine and electrostatic printers.

FIGS. 7A-B illustrates the printing plate current versus voltage for smooth wire and pin array corona units respectively.

FIGS. 8A-B illustrates the printing plate current versus the voltage on the plate for di-corotrons and scorotrons respectively.

FIG. 9 illustrates the plate/glass layout with its equivalent circuit.

FIGS. 10A-B illustrate electrical changes induced in printing plate during the transfer step.

FIG. 11 illustrates a mechanical schematic of a "flat" to "flat" printing apparatus.

FIG. 12 illustrates a cross section of a typical AC plasma display panel.

FIGS. 13A-C illustrate detailed sequences of manufacturing steps in the production of critical features of the AC plasma display.

FIGS. 14A-C illustrates the "self-printing" of the black intermatrix of a color filter panel

FIG. 14D illustrates the self-printing of a vacuum phosphor front panel.

FIGS. 15A-15F shows a six step process for producing a wafer with solder bumps

FIG. 16 shows a technique for building microstructures using a tiered printing plate.

FIG. 17 shows the steps subsequent to FIG. 16 in the microstructure building process.

FIG. 18 shows the process for making robust conductive lines of small width for various electronic applications.

FIG. 19 shows a side view of an apparatus for electrokinetic imaging of glass plates.

#### DETAILED DESCRIPTION OF THE PREFERRED EMBODIMENT

During the course of this description, like numbers will be used to identify like elements according to the different views which illustrate the invention.

FIG. 1 shows an overall mechanical schematic of the preferred embodiment. Drum 10 has a latent electrostatic image 13 on its surface 11. It is charged by sensitizing corona 12. If it is a photosensitive surface it is exposed in an imagewise fashion by LED/strip lens assembly 14. Alternately it could compose an electrostatic printing plate as disclosed by Reisenfeld of U.S. Pat. No. 4,732,831 where the image areas

retain charge and the background areas discharge before the drum 10 rotates to the developer unit 16. The unit 16 is comprised of toner developer roller 18 that are splashed with liquid toner by pipe 20. They rotate in such a manner as to move in the same direction of the drum but typically at a relative velocity of 1.5 times. Reverse roller 22 rotates in a manner opposite the drum 10 and with a relative velocity of 3 times. The purpose of this reverse roller 22 is to scavenge excess toner liquid off the image surface 11 which also controls unwanted background. A corona unit 24 at roughly the 5 o'clock position serves to "compact" the toner image before transfer. This is also referred to as "depress" corona.

Glass plate 26, which is pre-wetted with toner diluent, moves from right to left. It rests on insulating rollers 28 which are spaced with respect to the drum surface 11 to provide a nominal gap 42 between the glass surface 26 and the drum surface 11. Means are used to "float" either the image drum 10 with respect to the glass surface 26 or the glass surface 26 with respect to the drum 10, or glass 26, these are well known to those skilled in the mechanical arts. Corona unit 30 charges the bottom surfaces of the glass 26. Wire 31 is raised to about 7 kilovolts grounded mechanical shutters 32 are adjustable to charge the glass 26 at the proper desired location to achieve optimum toner transfer. Corona unit 34 is an AC corona discharge to discharge the drum 10 before cleaning. Alternately this unit, or a second AC corona, may be located after cleaning unit 36. This first AC corona is not shown.

Cleaning unit 36 typically consists of a squeegee roller 38 that does bulk, rough removal of residual toner, while wiper blade 40 does the final, complete cleaning of the drum surface 11. The drum 10 is now ready for the next image.

The arrangement of this system is modified in the embodiment shown in FIG. 19, wherein the planar substrate comprises a photopolymer coated glass on which an image is formed, which travels with respect to the toner supply, developer electrode and a cleaning roller, analogous to toner supply 18, 22; the drum 10; and the squeegee roller 38 of FIG. 10.

Important details of this embodiment are revealed by FIG. 2. Here is shown an enlarged view of the drum 10, gap 42, glass structure 26 at the transfer point, nominally at 6 o'clock. The drum 10 is wet with liquid toner 45 and excess liquid 51 coming into the nip formed by drum 10 and glass 26. The glass is pre-wetted with clear diluent to ensure that the gap between drum and glass is filled with liquid. Metering of liquid on the drum and the pre-wetting liquid on the glass is not very precise so a wave of excessive liquid 44 builds up in the input to the nip. This is referred to, herein, as the Tsunami effect. The toner on the drum before transfer 50 needs to transfer to the glass in a location of low turbulence, about 6 o'clock.

Alternately on the output end, the amount of liquid between drum and glass is precisely determined by the gap which is between 50 $\mu$  to 150 $\mu$  and can be easily controlled to +/- 5 $\mu$  with the "floating" techniques mentioned previously. Therefore a "film splitting" occurred as shown in FIG. 2 not necessarily 50%/50% as suggested by this drawing. Actual values will depend on the surface energy of the drum surface (amorphous selenium or silicon or alternately a photopolymer) versus that of the glass. For the purposes of this invention the film splitting point 46 is precisely defined and unchanging for particular materials and one gap setting while the wave front 44 is highly unstable and moves to the right from the beginning of the glass sheet to its end and can become quite violent and turbulent.

Important features of the preferred embodiment are now evident:

First: the actual electric fields for transfer can be quite large as typical soda lime glass has substantial electrical conductivity (as much as  $10^{-10}$  mho/cm) so the corona charge migrates through the glass to near the transfer point. As the drum and glass surface start moving away for each other very high electric fields can be generated.

Second: By moving the location of the corona and the shutters laterally, the exact location of the transfer "zone" can be moved with respect to the wave 44 and exit film splitting point 46. U.S. Pat. No. 4,849,784 by Blanchet-Fincher teaches the importance of not attempting gap transfer in the turbulence of the input wave.

Third: After transfer toner particles 48 are tightly bound to the surface of the glass by the internal transfer charges from the transfer corona. This prevents them from being smeared by random motion of residual diluent liquids on the glass before the toner is dried. Alternately if toner is transferred to a metal surface it is held to that surface by its "image" charge "seen" in the metal. This is classical electrostatic theory. Typically these "image" forces are significantly smaller than the strong binding forces between surface toner and the nearby transfer charges.

Other important features of this invention are the ability to print very large substrates, one meter by one meter or more with very small "features" (i.e. the dimensions of the image elements) and with very high levels of "overlay" accuracy (i.e. the registration of features) on one layer (or printing step) to overlay accurately the features on subsequent layers (or printing steps).

The electrostatic printing plate is shown in FIG. 3A is a photopolymer layer 52 bonded to an electrically grounded substrate 54. A photopolymer layer 52 is heat and pressure laminated to a grounded substrate, typically an aluminized polyester film (PET). It is then exposed through a contact photo tool to actinic radiation 65 (350 nm to 440 nm wavelength) to cross link the exposed areas 53. In FIG. 3B the plate is charged by a corona unit 56. The cross linked areas are much higher in electrical resistivity than normal photopolymer so they store charge for significant periods of time. After a suitable delay to allow the normal photopolymer to discharge 55, we have a latent image 62 on the printing plate as in FIG. 3C. In FIG. 3D a "reversal" development is effected with a liquid toner 58, i.e. development of the discharged areas of the plate (those referred to as normal photopolymer or not cross linked). Note the process can be a "normal" image, where the charged areas are developed or reversed as previously mentioned.

The Electrostatic Printing Plate can be film coated from a liquid solution which can be dried and partially hardened by a gentle bake. Coating methods include roller coating, spray coating, spin coating, dip coating or meniscus coating. Useful liquid photopolymers are usually negatively acting ones, those that cross link and that are insoluble in hydrocarbons or at least not significantly swelled by them. Typical examples of commercially available liquid materials are: Hoechst AZ-5200 IR, and MacDermid HDI-1, 2 or 3, also Mac Dermid. MT-1400. The dry film photopolymers are pre-cast films than can be heat and pressure laminated to suitable substrates. They include these materials:

DynaChem® AX 1.0 or 1.5, UF 0.5 or 1.0, 5032, 5038, 5050; MacDermid® SF-206, CF-1.3; DuPont Riston® 9512, 4615; both etch resist films and solder masks.

The liquid resists can range in thickness from a fraction of a micron to about  $15\mu$  to  $20\mu$ , depending on the coating technique used. They are typically in the fractional to  $15\mu$

range. The dry film resists tend to be much thicker in the  $13\mu$  to  $50\mu$  range; the ones of greatest interest here are  $25\mu$  to  $38\mu$  thick. But one requirement in flat panel manufacture is the generation of ever smaller features, in the  $10\mu$  to  $5\mu$  range. This presents some difficulty with resists in the  $30\mu$  to  $50\mu$  range; in the  $30\mu$  to  $50\mu$  range; less of a problem in the  $51$  to  $10\mu$  range.

An important feature of this invention is the partial exposure of the photo resist. Data has shown that the photopolymer 52 is exposed in ever increasing thickness of a layer 57 starting at its surface, as shown in FIGS. 4A through 4C. Increasingly by longer exposure to actinic radiation 65 cross-links ever deeper layer of the photo polymer. Therefore if one is using photopolymer at  $38$  micron thick but wants to make  $5\mu$  features, one might expose only one third 57a of it in thickness 57 as shown in FIG. 4D One now has highly resistive image in a "sea" of less resistive background areas. Since we never remove the unexposed background areas (and indeed their presence is a critical element in the success of the process, as discussed next), the partially exposed (or unexposed) layers under the image) present no problems. One determines the proper level of exposure for the "partial exposure" condition by a series of increasing exposure levels and measuring the charge voltage in large solid areas.

A second important feature of this invention is the need to keep the initial charge voltage on the exposed and unexposed regions to be either equal or within with in 50% of each other (i.e.  $V$  unexposed= $0.5$  V exposed). The reasons for this are subtle, but crucial, for the success of the process. FIG. 5A shows the ideal charge decay curves for the image elements 66 ( $V$  exposed= $f(t)$ ) and the background regions 68. ( $V$  unexposed= $f(t)$ ). Note after a short period of time there is no voltage in the background regions while the voltage and the image elements has decayed very little. While this is ideal and theoretically achievable in practice the initial charge voltage in the unexposed regions of the plate should be 50% or more of those values for the exposed regions as shown in FIG. 5B, exposed 70 and unexposed 72. The reason for this is a phenomenon called the "island effect". Basically a small spot of a good dielectric like PET sitting on a "sea" of bare copper cannot be charged to any significant value because of the electric field lines from the "island" to its surrounding "sea" which is at zero or grounded potential. These "field lines" direct incoming electric charge away from the image element and they land on the background areas.

Some photopolymers in the unexposed condition turn out to be "too" conductive and will not charge up to any significant value under the corona charge. Such plates when imaged by simple conditions will develop out the large image features but small image detail or fine structures are lost.

Such photopolymers can be used if one gives them a broad pre-exposure of the unexposed plate to bring it up to the proper electrical resistivity so that the initial voltage in the background areas is adequate. Then the pre-exposed plate is imaged with a photo-tool to produce a proper image above the pre-exposed level. This has been done in silver film halide for years and is called "pre-fogging" of the plate. Pre-exposure of an electrostatic printing plate is discussed in prior art literature such as Bujese in U.S. Pat. No. 4,968,570.

Other photopolymers have just the proper level of resistivity in the unexposed regions and require no pre-exposure or "pre-fogging". Some materials easily pick up moisture from the air and their intrinsic or unexposed resistivity depends upon their storage history and packaging. Generally these effects are not troublesome once known by the user and proper modern packaging and careful storage can yield a well defined photopolymer plate. Bench mark testing of each

## 11

batch of photopolymer will easily yield data to define proper exposure and "pre-fog" exposure if needed.

A third aspect of an optimized electrostatic printing process is the design and "type" of corona unit use as the charge corona. The machine design shown in the invention includes an AC erase discharge corona located just in front of the charge or sensitizing corona. By careful attention to design the AC corona will "reset" or discharge all areas of the plate after the print cycle. Now the plate is ready to be charged. Ideally the charging corona will charge all areas of the plate to the same voltage whether they be large solid areas of image, large areas of background (the unexposed regions) and the fine image structure.

There are basically four different structures used to make corona units in copiers and printers:

1. The familiar bare wire in a metallic shroud.
2. The unit "a" with an electrically biased metal screen or grid between it and the plate or drum (the Xerox trademark for this is a scorotron).
3. The glass coated wire driven by an AC signal in a "U" shaped shroud that has a DC bias, the dicrotron.
4. An etched metal "saw tooth" structure of corona emitting points.

The above approaches have different voltage versus corona current densities that will show which one is optimum for this situation. The electrostatic printing plate poses new problems for corona design. The plate has areas of two different electrical resistivities, the high resistivity charge retaining layer and the lower resistivity background regions. It has already been discussed how a plate could be pre-fogged to raise the background area resistivity to a point where its charge voltage would decay to a negligible value (typically 10% of the initial voltage) within the process time between charging and development. Given that this has been accomplished, the initial charge voltage in the non-exposed or background areas are a fraction of the initial voltage in the exposed areas and can be maximized by the choice of charge corona type and its design details. Procedures to accomplish this will now be described.

The various corona devices in use are shown in FIGS. 6A-6D. The top figure, FIG. 6A shows the oldest design dating to the late 1950's, the corona unit 74 or a bare wire usually gold plated tungsten of 50 $\mu$  to 75 $\mu$  in diameter in a grounded metal shroud. In some designs the front aperture was constricted inward to serve as a self extinguishing function in that the surface to be charged would not exceed a certain value. This was important otherwise the drum voltage, if excessive, could puncture the photo conductive surface of the drums used at that time, causing permanent damage.

An earlier version of the "pinched" design was the scorotron at the bottom of FIG. 6D. Here a metallic grid 76 structure in front of the corona wire is biased to a voltage perhaps 10% to 25% above the desired surface voltage (typically +800 for a 60 $\mu$  thick amorphous selenium layer).

The cost of the 1000 volt power supply to bias the grid structure and the assembly costs of the scorotron versus the corotron were the reason for the design of the "pinched-in" Corotron of FIG. 6A.

One problem with the simple corona unit is that in the negative mode the corona discharge is not positionally stable but moves back and forth randomly. One "fix" for this is to super-impose on the DC voltage to the corona wire, typically a ripple value of 10% to 20% of the DC. This causes the high intensity nodes of negative corona discharge to move down the wire at the AC frequency (usually 50 or 60 Hz). This simple, low cost solution was adequate for low speed copiers or printers, but when higher speed units were being designed, a new corona structure, the dicrotron 18 was invented, see

## 12

FIG. 6C. This used a glass coated wire which was driven by an ac voltage. The shroud (or shield) was biased to a DC voltage which would define whether positive or negative charge was extracted by the corona unit. This design has the advantages of a large diameter glass coated wires that was not easily "fouled" with random dust or toner particles. The bias power supply for the shield was also a low cost design. One unfortunate aspect of this design was that the dicrotron corona unit produced considerable levels of ozone. This trace gas is becoming unacceptable in the office environment, and must be neutralized.

That situation led to the design of the "pin corotron" 80 or a saw tooth edge 82 that is driven to a high voltage. With a properly made "saw tooth" the corona unit produced very uniform corona discharges, especially negative discharges. This corona unit has been highly successful in recent Xerox® organic photoreceptor machines. The important performance characteristic of a corona unit is the current to the plate to be charged versus the voltage to which the plate has charged. FIGS. 7A, 7B, 8A and 8B show these curves. Note that the wire and pin corotron have the same V-I curves FIG. 7A but that the AC curve FIG. 7B is quite different from the DC curve.

This invention uses an AC neutralizing corona unit to discharge the printing plate at the end of the printing cycle. Either the bare wire or pin corona are adequate for this job. The charging corona is located just after the neutralizing corona. Here a V-I curve is desired that will best charge the exposed and unexposed regions of the printing plate to the same voltage.

The ideal voltage-current characteristic from the corona unit would be one in which the corona current density (in microamps/cm<sup>2</sup>) would be independent of printing plate voltage, or a flat straight line in FIGS. 7A, 7B, 8A and 8B. Then if the plate is charged quickly, both exposed and unexposed plate areas would charge to the same value, after a suitable delay the unexposed regions would decay to a negligible value yielding an excellent electrostatic "contrast" (the difference between image and background).

Therefore, the best corotron design for this invention is the DC bare wire or pin corotron whose V-I curve is shown on FIG. 7A. Its V-I curves are the "flattest" of the four types of corona units and will yield the high ratio of unexposed to exposed initial charge voltage.

## Details of the Transfer Process

An important part of the invention relates to details of the transfer process not usually encountered in typical transfer processes to film and paper in the copying and laser printing industries. There toner, either liquid or dry is transferred to relatively thin webs of paper or polymeric film, typically 75 to 100 micron and in all cases the web is in virtual contact with the image surface.

In the invention toner images are transferred to relatively thick layer of glass, 0.5 to 3.0 mm thick (500 to 3,000 micron) spaced away from the image by a fluid filled mechanical gap of 50 to 150 microns. Relative conductivities of the glass versus the gap filling liquid (toner plus added diluent), capacitances, applied voltages and the time over which they are applied etc. are important.

FIG. 9 shows a mechanical schematic of the transfer process and a electrical equivalent circuit which allows one to calculate the voltage division across the three elements (glass 404, gap 410, and printing plate 400) during the transfer process.

A. Electrical Conductivity of the Glass Versus the Conductivity of the Gap Liquid

The most critical issues are the conductivities of the liquids in the gap versus the glass as this determines the voltage division between glass and gap. If most of the voltage appears across the glass and very little across the gap between plate and glass, all of toner will transfer. This is best illustrated by some examples:

Printing plate 400 consists of a photopolymer 402 of 10 to 50 micron thickness connected to electrical ground. Receiving glass plate 404 of typical thickness 0.5 to 3.0 mm thickness is backed by a field electrode 406 connected to transfer voltage 408. It is separated by mechanical gap 430 from printing plate 400. The equivalent circuit for this structure 412 is shown to the right.

A-1. A Glass of Interest is Electroviere ELC-7401-made in Switzerland.

If charged and then the voltage decay measured it shows a decay time constant of 1 second which calculates to a resistivity of  $2 \times 10^{12}$  ohm $\times$ cm. Typical ranges of toner bath conductivities are of the order 10 to 100 pico mho/cm ( $10^{11}$  to  $10^{10}$  ohm $\times$ cm $\times$ ms). There is one caveat to be disclosed. The charging test with the glass is a dc test and measures the flow of electronic charges through the glass, while the measure of toner conductivity is an 18 hertz test that measures back and forth flow of electrons, ions, and charged toner particles.

Now applying electromagnetic theory to the glass 404/gap 410 structure initially when a step function of voltage is applied 408 the voltages divide capacities between the elements, glass 404, gap 410, and plate 400. Since the imaged areas of the plate 400 are highly resistive they can be disregarded for short periods of time. Since the glass is thicker than the gap, typically 10 to 100 times, and it's dielectric constant is 5 versus 2.1 of the liquids in the gap, the voltages divided preferentially across the glass with little across the gap. If the conductivity of the gap fluids is higher than the glass in this situation will worsen the time and transfer will be inhibited.

With time, the voltages divide resistively between glass and gap. If the conductivity of the gap fluids is higher than that of the glass, practically all of the voltage is across the glass and none across the gap. If toner had transferred, it will back transfer due to the image charges on the printing plate. This, in fact has been observed.

A-2 Conductivity of the Diluent Used to Fill the Gap

Typically when a printing plate is imaged excess toner fluids are very effectively removed by a "reverse roller" that scavenges liquid containing random background particles; the result being an almost dry plate. Now the plate and glass are placed in proximity with each other and the gap between them filled with fluid. If one fills the gap with clear Isopar (conductivity less than 0.15 pmho/cm) the toner charge may be reduced by the lack of charge director in the clear Isopar. If one fills the gap with Isopar plus charge director with a conductivity of 20 pico mho/cm, the voltage division between glass and gap suffers. Again the demands of maintaining charge on the toner particles versus the conductivity of the gap fluids conflict. Conductive Isopar in the gap is desired but may not be possible if the glass has very high electrical resistivity.

Printing plates 430 and 432 in FIGS. 10A and 10B respectively are "negative" images of each other. 430 is cross linked in the image area and developed with toner 434 as shown in FIG. 15E. 432 is cross-linked in the non-image areas and developed with toner 434. Both plates are sensitized with charges 433. Field plates 436 are driven by voltages 438 and 440 respectively. Receiving glass 442 accepts the transferred

image. Mechanical gap 444 is filled with transfer fluid (not shown). High resistivity regions 446 are the cross-linked regions of the plate. Induced charges 448 occur when the transfer voltage is applied and are restricted to the non-cross linked regions of the plate.

B. Mounting Techniques for the Printing Plate and Glass

To preserve the fidelity of the toner image on the plate the transfer electric field must be everywhere normal to the plane of the plate and undistorted on the edges. And since we are 10 transferring to glass with a resistivity of the order of  $10^{12}$  to  $10^{16}$  ohm $\times$ cms., the mounting and holding of the plate must be consistent with these resistivities, i.e. these fixtures must be of materials substantially higher in resistivity. Even with the most conductive glass (lowest resistivity of  $10^{12}$  ohm $\times$  15 cms, some typical engineering materials, like cotton filled phenolics or poly acetals (Delrin of DuPont) may not be adequate for the job. For instance, Corning 7059 or 1737 glass is typically used for liquid crystal display panels for lap top computers. They have a resistivity of the order of  $10^{16}$  ohm $\times$  20 cm. A cotton filled phenolic resin material would not be adequate. Teflon type materials with resistivities of  $10^{18}$  are needed.

Also the conductivity of the bath can cause problems around the edges of the printing plate. Since the substrate of 25 the plate is electrical ground, the conductive gap filling liquids might distort the electric fields near the edges of the glass/plate assembly if they can contact electrical ground causing distorted image transfer.

C. Induced Charges in the Printing Plate During Image Transfer

An important feature of using the fixed resistivity configuration electrostatic printing plate is a phenomenon that helps to "focus" or direct the toner particles during transfer if the plate is used in the normal imaging mode. By this it is meant 35 that the toner development of the charged areas of the plate as opposed to the "reversal" mode where the discharged areas of the plate are developed with toner particles. The former is used in a typical office copier while the latter is used in a laser or LED printer.

40 Refer to FIGS. 10A and 10B. FIG. 10A shows the normal imaging mode, positive sensitizing charges developed with negative toner particles and transferred with a positive electric field. FIG. 10B shows reversal with again positive sensitizing charges, positive toner particles transferred with a 45 negative electric field. Note the charge retaining areas of the printing plate, they are highly resistive necessarily to retain the sensitizing charges. The other areas of the plate (areas not cross-linked in the plate exposure step) are much lower in resistivity.

50 During the transfer step, the transfer field "induces" electrical charges in these lower resistivity areas of the plate, which produces a significant result. Note the charge configuration in the "normal mode" plate, FIG. 10A. The sensitizing charges are positive while the induced background area 55 charges are negative. These background area negative charges enhance the strength of the imaging fields and help to control the direction of the toner particles during the transfer step. In the "reversal plate" (FIG. 10B), charges induced in the lower resistivity regions of the plate (the non-cross-linked regions) 60 are of the same polarity as the imaging fields and tend to reduce the fields. Indeed if the induced charge density equals that of the sensitizing charges there is no longer an imaging field and toner particles are free to move laterally during the transfer step. This will cause significant "de-focusing" of the 65 transferred toner image. For this reason, normal imaging is preferred when using the electrostatic printing plate for highest resolution images.

## 15

In summary, the electrostatic printing process for printing functional materials on glass plates is a simple one with few process steps. It has these advantages over current technologies:

1. It is a simple, direct process that proceeds at high rates, to 1 meter/sec.

2. It deposits a wide range of functional materials (conductors, insulators, phosphors, catalyst, etc.) to high definition or resolution with precise positional accuracy (called "overlay" accuracy in the silicon chip industry).

3. It prints on the glass surface without contact which has these advantages: a. mechanical tolerances are loosened in the design of production machinery b. previously printed materials are not disturbed c. it can print on a relief surface. In fact the invention can print a conductive line at the bottom of a 100 $\mu$  deep trench. d. the invention can coat the bottom and walls of the trench with a phosphor material or other applications not yet defined.

4. There is no photolithographic patterning of the glass.

5. There is no mechanical handling of the glass from step to step. We load a clean sheet of glass into the printing device and out comes a finished plate ready for sintering.

6. The process is a room temperature process until sintering so critical to large geometries due to thermal expansion of glass. In the printing of color filters, the four filter colors are printed at room temperature, then baked at once.

7. Expensive functional material is not wasted.

## First Alternate Embodiment of the Invention

FIG. 11 shows this embodiment Chuck 100 carrying electrostatic printing plate 102 is transported on linear bearings 104 by belt drive 106, canted at roughly a 45 degree angle to the horizontal. At the beginning of the print cycle chuck 100 starts at the top near pulley 108. Moving at uniform speed it passes corona unit 110 which charges the printing plate, 102 with a uniform electrostatic charge. After a short period of time, the low resistivity areas of the plate will discharge to a negligible charge level; the high resistivity areas of the plate retain the charge to near original levels. In an alternate process, if printing plate 102 is a photosensitive surface; it is exposed in an imagewise fashion by an optical means 111, such as an LED/strip lens assembly or scanned laser beam, after charging by the corona unit 110.

This latent electrostatic image is now developed by liquid toner which floods the gap between developer roll 112 and plate 102. Valve 114 floods this gap with a measured quantity of liquid toner 116. Developer roll 112 has an electrical bias voltage 118 which controls the accumulation of unwanted toner particles in background areas of the image. After passing between the developer roll plate 102 is stripped of excess liquids by reverse roll 120. After this the liquid toner is compacted by "depress" corona 122. The image is now finally developed and ready for transfer to the receiving substrate.

Receiving substrate 130, rests on its chuck 132 which rides on linear drive 134 driven by belts 136 and pulleys 138. It moves right past valve 140 which wets it with a thin layer of clear Isopar diluent. It moves to transfer position 148 and stops. Chuck 100 carrying printing plate 102 rotates approximately 135 degree counter clock wise to a position in obverse relation to receiving substrate 130. Spacing means not shown, accurately position plate 102 from receiving substrate 130 by a precisely controlled mechanical gap, typically of the order of 50 $\mu$  to 150 $\mu$ . A voltage is applied by a second corona unit 128 to chuck 132 to create a transfer electric field which transfers the toner image on plate 102 to receiving substrate 130.

## 16

Chuck 100 with printing plate 102 is now lifted vertically by means not shown or simply rotated clockwise by approximately 135 degree to its original position. Receiving substrate 130 is now dried before removing it from its chuck 132. Plate 102 is now moved up the 45° ramp and cleaned by suitable means, not shown, to repeat the next printing step.

The manifestation of the invention has advantages over the rotating process of the preferred embodiment in that is an asynchronous, i.e. variable time intervals can be introduced between each step of the process; and transfer occurs in the flat to flat situation when hydrodynamic events and forces have subsided. Furthermore, the flat receiving substrate, which may be of the order 1 m x 1.2 m must be on the bottom so it can be flooded by the diluent to fill the gap between the plate 102 and receiving substrate 130. Finally, the "overlay" accuracy of one flat plate, the printing plate; to a receiving sheet is much better, flat to flat, then in the dynamic situation of a moving flat sheet that needs to be accurately "phased" to a rotating print drum. Achieving very uniform linear and rotary drives are not trivial but phasing them "on the fly" to levels of their individual variations is a major task, all of which does not apply here.

## Second Alternate Embodiment

FIG. 12 shows a cross section of the cathode plate 200 of an AC Plasma Color Display Panel. It consists of a glass back plate 201 with black glass spacer ribs 202 that optically and electrically isolated image cells from one another. These ribs are typically 100 $\mu$  high and 30 $\mu$  to 40 $\mu$  in nominal width. At the bottom of the "wells" are the address electrode lines of copper 204 or nickel metal. Covering the walls and bottom of the "canyons" is the phosphor 206 that converts the UV radiation from the plasma discharge to visible radiation, red, green and blue, in the case of a color display. Alternate canyons are coated with red, then green then blue phosphor.

One advantage of the electrostatic printing technique is the non-contact or gap transfer aspect of it; i.e. the ability to transfer functional materials across relatively large mechanical gaps.

FIGS. 13A-13C show a greatly magnified picture of the mechanical gap 220 between the print drum and glass surface 200 of the invention. The gap here is set to a value of 150 $\mu$ . In the first manufacturing step shown in FIG. 13A, glass toner is printed to make the spacer/isolator ribs 202. Four layers of toner 203 are shown, each about 25 $\mu$  high, one printed on top of the other. The manufacturing sequence is as follows:

Step 1 Print first layer of glass ribs.

Step 2 Dry the toner by blowing warm air on it to partially set the resinous material that coats the glass particles. Note it is desired to maintain this as a constant temperature process so warm air is needed to compensate for the natural cooling that occurs with the evaporation of the diluent liquid.

Step 3 Reprint and dry the second layer of glass toner.

Step 4 Reprint and dry subsequent layers of glass toner until the desired height is achieved.

Step 5 Fire the glass panel at high temperature to burn off the resin in the toner and reflow the glass particles to make a solid rib.

Step 6 The rib manufacture process is now complete.

FIGS. 13A-13C show the process for the printing of the metallic address electrodes 204 in the base of the canyons formed by the ribs. A palladium catalytic toner 224 is imaged on the drum and transferred across the 150 $\mu$  gap to the base of the canyons, as shown in FIG. 13B. The toner is dried leaving a very thin layer of palladium seeds in a line that runs the length of the canyons. The plate is removed from the printing

machine of the invention and immersed in an "electro-less" plating bath. Metal growing from solution is on the palladium seeds, then on previously plated metal. Electroless processes have advanced to a point where one can plate up to one micron of metal per minute. After the growth of about  $25\mu$  of metal **216**, usually nickel, the cathode electrodes are complete.

FIG. 13C shows the deposition of phosphor toner **230** in the canyons. Phosphor toner **230** is imaged on the plate and transferred across the  $150\mu$  gap. Generally the transferred toner moves in straight lines but can coat relief images like coins. The toner image is sized to cover the walls of the canyons as well as the base where the electrodes are located. Note one phosphor color is imaged at a time so the printing plate has an image of every third canyon on it. After the first phosphor color **230** is imaged the toner is dried with warm air to set it; then the second color is imaged; then the third color. The same printing plate can be used for all three colors; all that is needed is to mechanically index the glass with respect to the printing drum. Cleaning of the drum must be adequate to prevent cross contamination.

The plasma display cathode plate is now finished. Glass ribs were built in 4 or 5 printing steps followed by a firing step to reflow the glass particles. Then electrodes were printed with a catalytic toner followed by an electro-less plating step. Finally three color phosphors were printed in the canyons formed by the glass ribs.

#### Third Alternate Embodiment

An alternate method to produce conductors is to print metal toners themselves, to burn off the resin that coats the metal particles; then reflow the metal into a smooth conductor pattern. Using the invention of the preferred embodiment one prints an aluminum toner onto the glass. The toner is then dried to temporarily fix it for reasons of safe handling. Now a rapid thermal processing of the metal is effected, where the toner and glass is raised to a temperature of  $50^\circ$  to  $100^\circ$  C. below the softening point of the glass (approximately  $500^\circ$  C. for soda lime glass). This effectively burns off the resin that coats the metallic particles. Now with an intense UV light source, the aluminum is heated to its melting point while the glass absorbs little UV energy. Aluminum which melts at  $659^\circ$  C. is a good choice of materials to be used with soda lime glass. Note this is not done in air but in a "reducing" atmosphere like one used in aluminum welding work.

#### Fourth Alternate Embodiment

In this embodiment the glass **300** in FIG. 14A is first coated with a thin, transparent layer **301** that is electrically conductive. This very thin layer is not shown. Indium Tin Oxide (ITO) is a possibility except it absorbs about 5 to 10% of the transmitted light and ITO processing is expensive, of the order of \$5 per square foot. The ITO conductivity of 50 to 100 ohms per square for a typical  $2\mu$  thick layer is higher than needed for this electrostatic process. A conducting polymer as resistive as  $10+5$  ohms per square is adequate for this electrostatic process, all that is needed is to establish an electrostatic ground plane **302** as shown in FIG. 14A.

In this case the coated glass **300** is imaged with the RGB color mosaics **304** which are then reflowed by final heating. The plate is now complete except for the black intermatrix which has yet to be produced. Transparent conductive layer is electrically grounded through edge contact **306** as shown in FIG. 14A. Now the entire plate is corona charged with a suitable corona generator **308** as in FIG. 14A. The conductive under layer discharges immediately, while the color mosaics

retain their charge **310** for considerable periods of time, as much as thousands of a second depending on the resins used in the mosaics. The partially finished color filter plate is now its own electrostatic printing plate, as seen in FIG. 14B. It can be developed in the reversal mode (i.e. develop the discharged [or uncharged] areas of the image) as is done in virtually all desk top laser printers.

In the example shown, the mosaics are charged positively so a toner with a positive charge **310** will develop the non-charged areas as in FIG. 14C. This black toner will produce the intermatrix between the mosaics. After the toner is dried, it will be reflowed by heating.

One of the principal advantages of this embodiment is that the final printing operation of the black intermatrix is self-correcting or "self-healing". Any image defects in the mosaics will be over-printed with black toner automatically. Also one does not need a high definition printing plate for the black intermatrix which must then be aligned to micron tolerances so as not to leave gaps between matrix and mosaic through which stray light will be passed. This self-correction feature is one of the greatest advantages of this embodiment

Another "self-printing" example as shown in this embodiment is seen in FIG. 14D. This glass plate #**330** is typical of the face plate of a field emission display (FED). The glass is first coated with black chrome oxide #**332** to enhance optical contrast and with a metallic chrome layer #**334** to conduct away to ground the electrons that hit the phosphor. It is desired to coat phosphor in the bare spaces on the glass surface between the chrome fingers which are all connected together. To "self-print" the phosphor toner the glass panel is placed on an electrically ground plate #**336**, chrome side up. Using a wire or metallic probe #**338** the chrome layer is made to act as an electrode by connecting it to a high voltage power supply, as high as possible before electrical breakdown occurs. Liquid toner is now poured over the plate and it is noted that toner #**340** "develops" on the bare glass areas by means of the fringing electrical fields. If the toner particles have a positive charge on them, a positive voltage must be connected to the chrome layer, with negative toner conversely a negative voltage with respect to ground is needed. As before open area defects in the chrome layer will have toner deposited on them in a "self-healing" manner.

#### Fifth Alternate Embodiment

According to a fifth alternate embodiment, a finished silicon wafer consisting of silicon substrate on which circuitry is constructed with electrode metal pads and a passivation layer between the electrodes, usually silicon nitride or polyimide resin. The wafer is coated with a photopolymer resin layer, which is patterned in known manner, to expose the metal pads. The patterned mask is now charged by means of a corona unit. Deposited charges will repel like charged toner particles into the holes.

The electrically charged mask is now developed with solder powder toner to develop the latent images, to produce relatively large toner piles. In the development step, the surface is flooded with toner having solder powder toner and diluent, from a large pipette. The trace of remaining background, if any occurs, is removed by inverting the solder bumped side of the wafer into a clear Isopar bath. The solder powder is then reflowed to form almost perfect spheres.

#### Sixth Alternate Embodiment

FIG. 15A shows a finished silicon wafer consisting of silicon substrate **420** on which circuitry is constructed (not,

shown) with electrode metal pads 424 and a passivation layer between electrodes 422, usually silicon nitride or polyimide resin. FIG. 15B shows the wafer coated with photopolymer resin layer 426, which is shown as pattern 428 in FIG. 15C. The patterning exposes the metal pads. The patterned mask is now charged by suitable means.

The electrically charged mask is now developed with solder powder toner (by means not shown) to develop images 432 as in FIG. 15E. Large toner piles are produced. The development step consists of flooding the surface of the wafer with solder powder toner and diluent from a large pipette. The trace of remaining background, if any occurs, is removed by inverting the solder bumped side of the wafer into a clear Isopar bath, not shown. The solder powder is now reflowed to form almost perfect spheres 434, as shown in FIG. 15F.

#### Seventh Alternate Embodiment

FIGS. 16 and 17 show a technique for building microstructures using electrostatic printing of liquid toners along with the tiered printing plate. Such microstructures are like the glass ribs in a plasma display panel. The photopolymer mask can be quite thick; 100, 120 or even several hundred microns thick. It is patterned according to the footprint of the desired structure. The patterned, tiered photopolymer mask is charged by appropriate means, like corona charging and for this instance the charge is negative. The toner particles, also negatively charged; are attracted into the trenches of the photo-polymer mask, filling it to the top, as in step 2, FIG. 17. The toner, as in the rib building case, is a glass flake coated with a sacrificial resin layer of acidic functionality (for negative charge).

The toner (resin coated frit) is consolidated into a stable mechanical structure by modest heating to reflow the resin coating thereby bonding the particles together (Step 3, FIG. 17). Then the mask is chemically stripped (also part of Step 3, FIG. 17). Finally the ribs are sintered at high temperatures to reflow the glass frit material (Step 4). The ribs are finished.

#### Eighth Alternate Embodiment

FIG. 18 shows the use of the photopolymer mask to produce fine metal traces of robust thickness; for example a 20 micron wide line, 5 or 6 microns thick. FIG. 18 shows perhaps a backplane for a flexible, flat panel display. The stainless steel substrate is coated with a thin dielectric layer for electrical isolation.  $\text{SiO}_2$  and  $\text{SiN}$  are preferred here but other insulating coatings like the polymers; polyimides, epoxies, the acrylics, etc. may also be also useful. A mask, liquid or dry film, is applied to the substrate. Note, the mask thickness matches the thickness of the trace desired. If shrinkage of the toner occurs upon sintering, the trace is typically 80% of the mask thickness. Again the mask is: (1) Patterned; (2) Charged; (3) Developed with metal toner; (4) The toner is sintered in place; (5) Optionally, the mask can be left in place or stripped by appropriate chemistry.

#### Example 1 of the Preferred Embodiment

An electrostatic printing plate was made by laminating DynaChem 5038, product of DynaChem Inc., Tustin Calif., photopolymer dry film resist material to 0.003 inches thick black anodized aluminum foil from Lawrence and Frederick of Des Plaines, Ill. (the part number is 1145-003-1419-SB). The laminating was done on an industry standard dry film laminator made by Western Magnum. After cooling from the

lamination process, the plate was exposed by a negative photo tool to nominal exposure level 100 millijoules/cm<sup>2</sup>.

The plate was charged to a nominal image voltage of -800V by a corona discharge unit. After about 2 seconds it was developed with a glass particle liquid toner by merely pouring the toner over it. Clear diluent (typically Isopar G®, Exxon Corp.) was used to wash away background particles. 125 $\mu$  thick spacers were placed on the plate edges and a glass plate wetted with diluent was placed over the spacers. Care was taken to ensure that no air bubbles were trapped in the space between the printing plate and the glass plate. The same corona unit was used to charge the top side of the glass plate with negative corona charges. The glass plate was lifted and an excellent glass toner image was found on the bottom surface of the glass plate. The glass was standard window glass (soda lime float glass) 0.090 inches thick.

#### Example 2 of the Preferred Embodiment

20 The glass toner of example 1, was prepared by the "organosol" process as taught by Kosel in U.S. Pat. No. 3,900,412. An organosol resin was polymerized in Isopar H diluent following the methods of Kosel. The resin had a Tg of -1°C and a core to shell ratio of 4. It was designated the nomenclature 25 of JB8-1 (Aveka Inc., Woodbury, Minn.) The toner contents were as follows:

75 g glass powder, Ferro Corporation, Cleveland, Ohio, #EG-2030-VEG  
25 g resin, JB8-1  
30 2 g ZrHexCem, OMG Americas, Cleveland, Ohio, Prod. Cd. 949  
300 g of Isopar L®, Exxon Corporation

It was processed for one hour in a Disperamat F105® vertical bead mill made by Byk-Gardner Incorporated of 35 Germany. Processing was done at medium speed. The resulting toner had the following characteristic:  
mean particle size 1.27 $\mu$   
toner conductivity 9.9 pico mho/cm  
particle mobility 3.06 $\times 10^{-6}$  m<sup>2</sup>/v-s  
40 Z (or zeta) potential 14.7 millivolts

The glass particles have a true mass density of 5.2 while the Isopar L® has a density of 0.8 so the toner settles out substantially in 15 to 30 minutes. It can be successfully re-dispersed by moderately shaking of the toner containers by hand.

#### Example 3 of the Preferred Embodiment

Example #1 was repeated with the toner of example #2 but 50 the toner was transferred to Cr coated glass. 75 mm $\times$ 75 mm $\times$ 1.2 mm Corning 7059® glass were sputter coated with 100 nm to 150 nm of pure chrome. The resulting surface had a brilliant shine to it. The Cr surface on the glass was wetted with Isopar and this wetted glass placed on the PET on a 55 developed printing plate. The Cr surface was connected to a lab supply producing -1600V. Good glass toner images were transferred on the Cr coated glass. The PET spacers were 125 $\mu$  thick.

#### Example 4 of the Preferred Embodiment

A catalytic toner was prepared with the following ingredients:  
2 g of Palladium powder, Aldrich Chemical #32666-6  
65 17 g of organosol resin, JB-8-1  
1 g of ZrHexChem  
100 g of Isopar L

## 21

The mixture was dispersed in the vertical bead mill for 1.5 hours at 2,000 rpm. The resulting toner had these measured characteristics:

mean particle size  $0.333\mu$  conductivity 169 p mho/cm

The toner was imaged using the plate of Example 1 and transferred to soda lime glass plates. These plates were dried then put into an electroless copper bath (typically Shipley CuPosit™ 328, Shipley Inc, Marlboro Mass.) for 10 minute at  $23^{\circ}\text{C}$ . Significant copper metal was visible on the glass surface.

## Example 5 of the Preferred Embodiment

An aluminum powder toner was prepared by the following formulas:

75 g of Alex Al, Argonide Corp.

25 g of organosol resin JB-8-1

2 g of ZrHexChem

350 g Isopar L

The mixture was dispersed for 1.5 hours in the vertical bead mill and the resulting toner specifications were:

mean particle size  $30\mu$

mobility  $6.95 \times 10^{-11} \text{ m}^2/\text{v}\cdot\text{s}$

conductivity 40 p mho/cm

zeta potential 5.314 mV

The toner was imaged on the plate of example 1 and transferred to the same type to soda lime glass. After drying it was subjected to rapid thermal processing in the model CP-3545 RTP machine of Interact of Rocklin, Calif. The toner and glass were pre-heated to  $550^{\circ}\text{C}$ . in a non-oxidizing atmosphere. It was then exposed to intense UV radiation that heated the aluminum toner but not the glass.

## Example 1 of the First Alternate Embodiment

A printing plate from 38 micron thick DynaChem 5038 photopolymer was charged and imaged with Indigo E-1000 toner with a concentration of 1.5% by weight and a conductivity of 25 pico mhos/cm. Corning 7059 glass 1 mm thick was placed on PET film, 25 microns thick spacers, above the plate. The gap between glass and plate was filled with pure Isopar G whose conductivity is less than 0.15 pico mho/cm. An electrode was placed on top of the 7059 glass and excited to  $+10\text{ kV}$  with respect to the grounded base of the printing plate. The transfer voltage was held for 10 minutes.

The glass was removed with the transfer voltage still applied and it was noted that no toner transferred. This shows that virtually all of the voltage appeared across the glass and none or little across the gap so no toner transferred.

Initially toner may have transferred to the glass due to the capacitive division of voltages between glass and gap (theoretically about 12% of the  $10\text{ kV}$  or  $1200\text{ v}$ ), but as the voltage across the gap collapses, the toner would back transfer to the plate.

## Example 2 of the First Alternate Embodiment

The plate of Example 1 of the First Alternate Embodiment was imaged and developed. Electrovere glass ELC-7401 with a resistivity of  $2 \times 10^{12} \text{ ohm}\cdot\text{cm}$  was placed on 50 micron thick PET spacers. The gap between glass and plate filled with Isopar G spiked with Indigo Imaging Agent to a conductivity of 12.4 pico mho/cm. A transfer voltage of  $4\text{ kV}$  was applied to the top of the Electrovere glass for 5 seconds while linearly reducing it to  $3\text{ kV}$ . The glass was removed with the  $3\text{ kV}$  transfer voltage still applied.

## 22

An excellent image was seen on the glass with very good edge acuity. The image was superior to a similar image created using just clear Isopar G (i.e. very low conductivity) to fill the gap. Demonstrating that the charges, on the toner particles, are better preserved with the conductive, gap filling liquid.

## Example 3 of the First Alternate Embodiment

10 An image was created on the plate of Example 1 of the First Alternate Embodiment using that toner. 2.25 mm thick soda lime float glass (i.e. common window glass) was placed on 50 micron PET spacers, above the plate. Isopar G® conductivity treated with Indigo Imaging Agent to a conductivity of 25 pico mho/cm was used to fill the gap between glass and plate. An electrode connected to  $5\text{ kV}$  of voltage was placed on top of the plate, which was reduced to  $3\text{ kV}$  in 5 seconds. The glass plate was lifted and an image of low density was found on the glass. A significant amount of toner remained untransferred on the printing plate. The conductivity of the gap liquid reduced the effective voltage across the gap causing poor transfer.

15 If clear Isopar G® is used good, complete transfer occurs though edge acuity may suffer. With this moderately resistive glass (of the order  $10^{+13} \text{ ohm}\cdot\text{cm}$ ), the conductive Isopar® in the gap reduces the voltage across the gap resulting in incomplete transfer.

## Example 1 of the Fourth Alternate Embodiment

20 A 1.1 mm thick plate of soda lime glass was patterned with black chrome oxide, then metallic chrome with phosphor openings of  $60\mu$  by  $130\mu$  in a solid pattern of  $75\text{ mm} \times 100\text{ mm}$ . The plate was placed, chrome side up on a grounded copper plate. Electrical contact was made with the chrome surface and the power supply was turned on to  $+6,000$  volts. No break down occurred. The chrome surface was flooded with the phosphor containing toner Similar to Example #2, the difference was equal amounts of phosphor and resin, 50 g of phosphor, 50 g of JB8-1. Unwanted background was washed away with clear Isopar G®. The plate was allowed to air-dry at room temperature. Good phosphor toner images were noted in the clear spaces between the chrome fingers. The phosphor toner NP-1053A was obtained from Nichia Kagaku Kogyo, 25 K. K., Tokashima-ken, Japan.

## Example 1 of the Sixth Alternate Embodiment

30 We will first describe a method for imparting a coating to the particles. In preparing particles for coating it may become necessary to remove the fine particles from the bulk in order to reduce the amount of agglomerates occurring during the coating process. One way to accomplish this is by introducing the material to one or more washes where the material is 35 agitated in fluid such as de-ionized water, Isopar® linear, aliphatic hydrocarbon or any other suitable fluids/solvents. After the mixture has been stirred sufficiently it will be allowed to settle for a pre-determined time (based on the density of the material) and then the diluent will be decanted. 40 Additional washes may give the desired results. After washing the diluent is decanted and the material is oven-dried.

45 One approach to making functional particles into toners is to coat them with a resin that has either an acidic or basic functionality necessary for the electrochemical reactions to form the toner particles charge. A measured amount of functional material having a known particle size, hence a known surface area per unit weight, will determine the amount of

resin needed to impart a desired thickness of coating on the particle. Coating the material requires it to be placed in an amount of solvent which is the same solvent as that which dissolves the resin. While agitating/stirring this solution the metered resin-solvent solution is added and after a pre-determined time Isopar® is added and the entire mixture is heated to approx. 60° C. for some time to evaporate sufficient amounts of resin solvent., then cooled to ambient while stirring to eliminate all of the resin's solvent. Other methods of solvent extraction may be available. The Isopar® diluent is then decanted and the coated particulate material is collected and washed several times. It is now ready to be made into a liquid toner.

#### Example 2 of the Sixth Alternate Embodiment

15 g of glass frit material (Spheriglass 5000, Potter Industries; Carlstadt, N.J.) was added into 80 g. Isopropyl alcohol (the solvent for the resin) and stirred while adding 1.8 g of resin dissolved in IPA (20% by weight). This mixture is stirred for 5 minutes and 112 g of Isopar G® is added and stirred for 30 mins. This mixture, while stirring, is then raised in temperature to 60 deg C., for 2 hours; then allowed to cool for 4 hrs. The diluent is decanted and the coated glass frit is washed two times in Isopar G®. Suitable resins include, Sylprint S-8200 (Arizona Chemical, Jacksonville FL.) and SAA-100 (Lyondell Chemical, Houston, Tx.).

#### Example 3 of the Sixth Alternate Embodiment

To make the resin coated glass frit into a functional liquid toner, a carrier liquid such as Isopar G is used. 1 to 5 g of coated frit is dispersed in 100 g of Isopar G® (Exxon/Mobil, Houston, Tx.) with a suitable polyelectrolyte (charge director) to achieve a bath conductivity of 6 to 8 pico mhos per cm. (typically 9 drops of 10% solution of basic barium petronate in Isopar G®). This formulae makes a good negatively charged toner with the acidic resin S-8200. With the basic SAA-100, one needs to use the charge director #12-76 (Hunt Imaging, Berea. Oh.) to make a positively charged toner.

#### Example 4 of the Sixth Alternate Embodiment

Type 5 solder, 63/37 Sn/Pb in the 10 to 30 micron range is coated with Sylprint S-8200 in a fluidized bed coater (Worster process, The Coatings Place; Verona Wis.). 120 g of this powder is dispersed in 1 liter of Isopar G® with 6 ml of Indigo Imaging Agent., cut 10:1 in Isopar G®. It is stirred by a magnetic stirrer before use for about 4 hrs.

#### Example 5 of the Sixth Alternate Embodiment

A finished silicon wafer is roll laminated with Dynamask 5040 (Morton Inc.; Tustin, Cal) a 100 micron thick dry film solder mask. After exposure and development, the cross-linking reaction is completed by a post-exposure of approx. 1 joule per cm sq. of actinic energy and a bake cycle of 150 C for 90 mins.

This mask is charged to -800 v to -1,000 v and developed with the toner of Example 4 of the Sixth Alternate Embodiment. Excellent bumps are produced. This mask is then stripped with Florida Cir Tek Inc, RS-3150 (Cir Tek, Boulder Co.).

#### Example 6 of the Sixth Alternate Embodiment

The dry film photo-polymer of Example 5 of the Sixth Alternate Embodiment is replaced with liquid photopolymer

HD-4000, a photo-imaginable polyimide resin, yielding coating in the 75 to 100 micron range. All other test conditions remain the same. This polyimide resin which is very durable and inert is not stripped but left intact.

5 In summary, this invention comprises a relatively uncomplicated high yield manufacturing process in which functional materials are configured as liquid electrographic toners that can be printed at commercially interesting rates of production in a non-contact mode. This non-contact feature 10 allows one to print on non-flat surfaces or even relief surfaces such as ribbed surfaces.

While the invention has been described with reference to the preferred embodiments thereof it will be appreciated that various modifications can be made to the parts and methods 15 that comprise the invention without departing from the spirit and scope thereof.

What we claim is:

1. A method for building microstructures, comprising the steps of:

20 (a) forming a patterned dielectric mask on a substrate, having a mask thickness equal to or larger than a desired height of a microstructure to be formed, and relief features formed into the mask;  
 (b) applying a first spatial electrical charge to the patterned dielectric mask, to thereby form a first spatial charge pattern;  
 (c) developing the first spatial charge pattern with an electrically charged first functional toner in a liquid;  
 (d) applying a second spatial electrical charge to the patterned dielectric mask, to thereby form a second spatial charge pattern;  
 (e) developing the second spatial charge pattern with an electrically charged first functional toner in a liquid, superposed on the developed first functional toner; and  
 (f) processing the first and second functional toner material 30 to form useful microstructures corresponding to the relief features of the patterned dielectric mask, wherein a composition of the microstructures varies in dependence on the first and second spatial charge distributions.

35 2. The method for building microstructures according to claim 1, wherein at least one of the first and second functional toners deposited on the patterned dielectric mask comprises a first portion of a higher melt point glass mixed with a second portion of a lower melt point material that, during said processing, is heated to a temperature that causes at least the lower melt point material to re-flow and to bond the higher melt point material together, while still retaining shape of the microstructure prior to the re-flow.

40 3. The method according to claim 2, wherein the first portion is present in a greater quantity than the second portion, the first and second portions comprising a majority of a solids portion of the at least one of the first and second functional toners deposited on the patterned dielectric mask.

45 4. The method according to claim 1, wherein at least one of the first and second functional toners in a respective liquid comprises metal particles coated with an organic-metallic composition suspended in the respective liquid, wherein said processing step comprises decomposing the organic-metallic composition under heat, to thereby sintering the metal particles together, wherein the sintered metal particles correspond in shape to the patterned dielectric mask.

50 5. The method according to claim 1, wherein at least one of the first and second functional toners in a respective liquid 55 comprises inorganic particles coated with an organic-metallic composition suspended in the respective liquid, wherein said processing step comprises heating, the organic-metallic com-

## 25

position decomposing as a result of the heating, a decomposition product of the organic-metallic composition sintering the inorganic particles together, wherein the metal particles correspond in shape to the patterned dielectric mask.

6. The method according to claim 1, wherein at least one of the first and second functional toners comprises particles, each comprising a particle core composition coated with a particle shell composition, the particle shell composition transforming in said processing step to form a solid matrix with the particle core composition, wherein the solid matrix corresponds in shape to the patterned dielectric mask.

7. The method according to claim 1, wherein said processing step comprises at least one step selected from the group: exposing the developed first and second functional toners deposited on the patterned dielectric mask to actinic radiation to initiate or maintain a decomposition reaction; exposing the developed first and second functional toners deposited on the patterned dielectric mask to at least heat to initiate or maintain a decomposition reaction; exposing the developed first and second functional toners deposited on the patterned dielectric mask to at least an chemical reactant provided external to the first and second functional toner material, to initiate or maintain a decomposition reaction; and transforming the first and second functional toners deposited on the patterned dielectric mask through at least temporary change of state between solid, liquid and gas.

8. The method according to claim 1, wherein said processing step comprises a polymerization reaction.

9. The method according to claim 1, wherein the processed first and second functional toners deposited on the patterned dielectric mask comprises a material having a reflow temperature, wherein the material is reflowed to form conductive spheres due to surface tension forces.

10. The method according to claim 1, wherein the first and second functional toners deposited on the patterned dielectric mask comprises particles having a core having a high melting temperature, a mantle having a low melting temperature, and a crust having surfactant properties, wherein said processing step removes at least a portion of the crust and maintains a temperature between a melting temperature of the mantle and the crust, to thereby adhere the particles into a matrix.

11. The method according to claim 1, wherein the spatial charge pattern defines at least one rib, which after said processing has a length at least three times longer than a width thereof.

12. The method according to claim 1, wherein the spatial charge pattern defines at least one barrier at least partially surrounding a physical feature of the substrate.

13. The method according to claim 1, wherein the first and second functional toners deposited on the patterned dielectric mask comprises a glass type frit, wherein said processing step fuses the frit into a fused glass structure on the substrate.

14. The method according to claim 1, wherein the microstructures comprise conductive metal structures having a section height greater than a respective section width.

15. The method according to claim 1, wherein the substrate is non-planar, and the processed microstructures are non-planar.

16. The method according to claim 1, wherein the substrate comprises a plurality of existing microstructures, and wherein the processed microstructures are formed superposed on the plurality of existing microstructures.

17. The method according to claim 1, wherein said selectively applying, developing, and processing are sequentially repeated for the first and second functional toners, wherein after an initial processing, the substrate comprises a plurality of existing microstructures formed of the processed first func-

## 26

tional toner comprising a first material composition, and wherein the processed microstructures in a subsequent processing are formed of the processed second functional toner comprising a second material composition, to thereby produce a plurality of processed microstructures having different respective material composition.

18. The method according to claim 1, wherein said developing step comprises:

partially developing the charge pattern with the electrically charged first functional toner in a respective liquid; and then

partially developing the charge pattern with the electrically charged second functional toner in a respective liquid, to thereby produce at least one unprocessed microstructure having a spatially varying composition, which is then processed to form a microstructure having a spatially varying composition.

19. The method according to claim 1, wherein the charge on the patterned mask can be selectively applied according to a plurality of distributions, said process comprising the steps of:

applying a first spatial charge distribution to the patterned dielectric mask;

developing the first spatial charge pattern with the electrically charged first functional toner in a respective liquid; applying a second spatial charge distribution to the patterned dielectric mask;

developing the second spatial charge pattern with the electrically charged second functional toner in a respective liquid, superposed on the developed first functional toner;

processing the superposed first and second functional toner to form a microstructure, wherein a composition of the microstructure varies in dependence on the first and second spatial charge distributions.

20. The method according to claim 19, wherein the developed first functional toner deposited on the patterned dielectric mask is at least partially processed prior to developing with the second functional toner.

21. The method according to claim 1, wherein said developing step comprises:

partially developing the charge pattern with the electrically charged first functional toner in a respective liquid to incompletely fill the patterned mask; and then

developing the charge pattern with the electrically charged second functional toner in a respective liquid to finish filling the patterned mask,

to thereby produce a layered microstructure.

22. The method according to claim 1, further comprising the step of removing the patterned dielectric mask without disturbing the formed microstructure.

23. The method according to claim 1, wherein the substrate is a thin dielectric, further comprising providing a conductor on an opposite side of the substrate from the dielectric mask, and imposing a charge on the conductor, to thereby form the spatial charge pattern.

24. A method of forming a microstructure, comprising a substrate and at least two different electronically functional toner materials selectively formed into a pattern on the substrate, the microstructure comprising at least one electrically conductive element, comprising:

(a) forming a patterned dielectric photopolymer mask on the substrate, having a mask thickness equal to or larger than a height of a microstructure to be formed, and having relief features formed into the mask;

**27**

- (b) electrostatically charging the patterned dielectric mask in at least two different patterns at different times, to thereby form at least two different spatially varying electrostatic charge patterns in dependence on at least the relief features formed into the mask;
- (c) developing the spatial charge pattern at the different times, with the at least two electronically functional toner materials, each in a respective dielectric liquid, to selectively deposit the at least two different functional

5

**28**

- toner materials in dependence on the different spatial charge patterns; and
- (d) processing the deposited at least two different functional toner materials to form a microstructure dependent on at least the relief features of the patterned dielectric mask.

\* \* \* \* \*